



US007997950B2

(12) **United States Patent**  
**Wei et al.**

(10) **Patent No.:** **US 7,997,950 B2**  
(b5) **Date of Patent:** **\*Aug. 16, 2011**

(54) **FIELD EMISSION ELECTRON SOURCE HAVING CARBON NANOTUBES AND METHOD FOR MANUFACTURING THE SAME**

(75) Inventors: **Yang Wei**, Bei-Jing (CN); **Zhuo Chen**, Bei-Jing (CN); **Liang Liu**, Bei-Jing (CN); **Shou-Shan Fan**, Bei-Jing (CN)

(73) Assignee: **Hon Hai Precision Industry Co., Ltd.**, Tu-Cheng, New Taipei (TW)

(\*) Notice: Subject to any disclaimer, the term of this patent is extended or adjusted under 35 U.S.C. 154(b) by 384 days.

This patent is subject to a terminal disclaimer.

(21) Appl. No.: **12/006,334**

(22) Filed: **Dec. 29, 2007**

(65) **Prior Publication Data**

US 2009/0115306 A1 May 7, 2009

(30) **Foreign Application Priority Data**

Nov. 2, 2007 (CN) ..... 2007 1 0124240

(51) **Int. Cl.**

**H01J 9/00** (2006.01)

**H01J 9/04** (2006.01)

(52) **U.S. Cl.** ..... **445/50; 445/49; 445/51**

(58) **Field of Classification Search** ..... **445/49, 445/50, 51**

See application file for complete search history.



(56)

**References Cited**

**U.S. PATENT DOCUMENTS**

|                   |         |                             |
|-------------------|---------|-----------------------------|
| 7,586,249 B2      | 9/2009  | Jiang et al.                |
| 7,704,480 B2 *    | 4/2010  | Jiang et al. .... 423/447.2 |
| 2003/0186625 A1 * | 10/2003 | Nakayama et al. .... 451/28 |
| 2004/0095050 A1   | 5/2004  | Liu et al.                  |
| 2007/0145878 A1   | 6/2007  | Liu et al.                  |
| 2007/0166223 A1   | 7/2007  | Jiang et al.                |
| 2008/0170982 A1   | 7/2008  | Zhang et al.                |
| 2009/0239439 A1 * | 9/2009  | Wei et al. .... 445/46      |

**FOREIGN PATENT DOCUMENTS**

|    |                   |         |
|----|-------------------|---------|
| CN | 1501422 A         | 6/2004  |
| CN | 1941249 A         | 4/2007  |
| CN | 1982209 A         | 6/2007  |
| CN | 1988108 A         | 6/2007  |
| CN | 101007366 A       | 8/2007  |
| JP | 2003502798        | 1/2003  |
| JP | 2004303521        | 10/2004 |
| WO | WO0077813         | 12/2000 |
| WO | WO2007015710      | 2/2007  |
| WO | WO2007015710 A2 * | 2/2007  |

\* cited by examiner

*Primary Examiner* — Nimeshkumar Patel

*Assistant Examiner* — Anthony Perry

(74) *Attorney, Agent, or Firm* — Altis Law Group, Inc.

(57) **ABSTRACT**

A field emission electron source having carbon nanotubes includes a CNT string and a conductive base. The CNT string has an end portion and a broken end portion, the end portion is contacted with and electrically connected to the surface of the conductive base. The CNTs at the broken end portion form a tooth-shape structure, wherein some CNTs protruding and higher than the adjacent CNTs. Each protruding CNT functions as an electron emitter. Further, a method for manufacturing a field emission electron source is provided. The field emission efficiency of the field emission electron source is high.

**15 Claims, 8 Drawing Sheets**





FIG. 1



FIG. 2



FIG. 3



**FIG. 4**



FIG. 5



FIG. 6



FIG. 7



FIG. 8

## 1

**FIELD EMISSION ELECTRON SOURCE  
HAVING CARBON NANOTUBES AND  
METHOD FOR MANUFACTURING THE  
SAME**

RELATED APPLICATIONS

This application is related to commonly-assigned, co-pending application: U.S. patent application Ser. No. 12/006,305, entitled "METHOD FOR MANUFACTURING FIELD EMISSION ELECTRON SOURCE HAVING CARBON NANOTUBE", filed Dec. 29, 2007 and U.S. patent application Ser. No. 12/006,335, entitled "METHOD FOR MANUFACTURING FIELD EMISSION ELECTRON SOURCE HAVING CARBON NANOTUBE", filed Dec. 29, 2007. The disclosure of the respective above-identified application is incorporated herein by reference.

BACKGROUND

1. Field of the Invention

The invention relates to field emission electron sources and methods for manufacturing the same and, particularly, to a field emission electron source having carbon nanotubes and a method for manufacturing the same.

2. Discussion of Related Art

Carbon nanotubes (CNTs) produced by means of arc discharge between graphite rods were first discovered and reported in an article by Sumio Iijima, entitled "Helical Microtubules of Graphitic Carbon" (Nature, Vol. 354, Nov. 7, 1991, pp. 56-58). CNTs also feature extremely high electrical conductivity, very small diameters (much less than 100 nanometers), large aspect ratios (i.e. length/diameter ratios) (greater than 1000), and a tip-surface area near the theoretical limit (the smaller the tip-surface area, the more concentrated the electric field, and the greater the field enhancement factor). These features tend to make CNTs ideal candidates for field emission electron sources.

Generally, a field emission electron source having CNTs includes a conductive base and CNTs formed on the conductive base. The CNTs acts as emitter of the field emission electron source. The methods adopted for forming the CNTs on the conductive base mainly include mechanical methods and in-situ synthesis methods. The mechanical method is performed by respectively placing single CNT on a conductive base by an Atomic force microscope (AFM), then fixing CNT on the conductive base by conductive pastes or adhesives. However, the controllability of the mechanical method is less than desired, because single CNT is so tiny in size.

The in-situ synthesis method is performed by coating metal catalysts on a conductive base and synthesizing CNTs on the conductive base directly by means of chemical vapor deposition (CVD). However, the mechanical connection between the CNTs and the conductive base often is relatively weak and thus unreliable. In factual use, such CNTs are easy to be drawn away from the conductive base due to the electric field force, which would damage the field emission electron source and/or decrease its performance. Furthermore, the shield effect between the adjacent CNTs may reduce the field emission efficiency thereof.

What is needed, therefore, is a field emission source employing CNTs, which has a firm mechanical connection between CNTs and the conductive base, and has a high field emission efficiency, and a controllable method for manufacturing the field emission source.

SUMMARY

A field emission electron source having carbon nanotubes includes a CNT string and a conductive base. The CNT string

## 2

has an end portion and a broken end portion, the end portion is contacted with and electrically connected to the surface of the conductive base. The CNTs at the broken end portion form a tooth-shape structure, wherein some CNTs protruding and higher than the adjacent CNTs.

10 A method for manufacturing a field emission electron source includes: providing a CNT array; drawing a number of CNT bundles from the CNT array to form a CNT yarn; soaking the CNT yarn into an organic solvent, and shrinking the CNT yarn into a CNT string after the organic solvent volatilizing; irradiating a predetermined point of the CNT string with a laser beam; applying a voltage between two opposite ends of the CNT string, until the CNT string snapping; and attaching the snapped CNT string to a conductive base, and achieving a field emission electron source.

20 Compared with the conventional field emission electron source, the present field emission electron source has the following advantages: firstly, a CNT string, which is in a larger scale than the CNT, is used as the electron emitter, and thus the CNT string is more easily controlled. Secondly, the CNT string is attached to the conductive base by a conductive paste, and thus the connection is stable. Thirdly, the broken end portion of the CNT string is in a tooth-shape structure, 25 which can prevent from the shield effect caused by the adjacent CNTs. Further, the CNT string is snapped by applying a voltage thereon, the electric and thermal conductivity, and mechanical strength of the CNT string can be improved. Therefore, the field emission efficiency of the field emission electron source is improved. Fourthly, by a laser beam irradiation, the location of the CNT string snapping can be precisely controlled, and thus the field emission electron source can be easily manufactured.

30 Other advantages and novel features of the present ion source element will become more apparent from the following detailed description of preferred embodiments when taken in conjunction with the accompanying drawings.

BRIEF DESCRIPTION OF THE DRAWINGS

40 Many aspects of the present field emission electron source and the present method for manufacturing the same can be better understood with reference to the following drawings. The components in the drawings are not necessarily to scale, 45 the emphasis instead being placed upon clearly illustrating the principles of the present field emission electron source and the method for manufacturing the same.

FIG. 1 is a schematic, cross-sectional view, showing the present field emission electron source.

50 FIG. 2 is a schematic, amplificatory view of part II in FIG. 1.

FIG. 3 is a Scanning Electron Microscope (SEM) photo, showing part II in FIG. 1.

FIG. 4 is a Transmission Electron Microscope (TEM) 55 photo, showing part II in FIG. 1.

FIG. 5 is a process chart showing the steps of the method for manufacturing the present field emission electron source.

FIG. 6 is a schematic view, showing a laser beam irradiating a carbon nanotube string.

60 FIG. 7 is a Raman spectrum of the broken end portion of the present field emission electron source.

FIG. 8 is a current-voltage graph of the present field emission electron source.

65 Corresponding reference characters indicate corresponding parts throughout the several views. The exemplifications set out herein illustrate at least one preferred embodiment of the field emission electron source and the method for manu-

factoring the same, in one form, and such exemplifications are not to be construed as limiting the scope of the invention in any manner.

#### DETAILED DESCRIPTION OF PREFERRED EMBODIMENTS

Reference will now be made to the drawings to describe the preferred embodiments of the present field emission electron source and the present method, in detail.

Referring to FIG. 1, a field emission electron source 10 includes a CNT string 12 and a conductive base 14. The CNT string 12 includes an end portion 122 and a broken end portion 124. The CNT string 12 is attached to the conductive base 14 with the end portion 122 being in contact with and electrically connected to the surface of the conductive base 14. The included angle between the longitudinal axis of the CNT string 12 with the surface of the conductive base 14 can be equal to or greater than 0 degree and equal to or less than 90 degrees.

The CNT string 12 is composed of a number of closely packed CNT bundles, and each of the CNT bundles includes a number of CNTs, which are substantially parallel to each other and are joined by van der Waals attractive force. A diameter of the CNT string 12 is in an approximate range from 1 to 100 microns ( $\mu\text{m}$ ), and a length thereof is in an approximate range from 0.1-10 centimeters (cm). Referring to FIGS. 2, 3 and 4, the CNTs at the broken end portion 124 form a tooth-shaped structure, i.e., some CNTs protruding and higher than the adjacent CNTs. The CNTs at the broken end portion 124 have smaller diameter and fewer number of graphite layer, typically, less than 5 nanometer (nm) in diameter and about 2-3 in wall. However, the CNTs in the CNT string 12 other than the broken end portion 124 are about 15 nm in diameter and more than 5 in wall. The conductive base 14 is made of an electrically conductive material, such as nickel, copper, tungsten, gold, molybdenum or platinum, or an insulated base with a conductive film formed thereon.

Referring to FIG. 5, a method for manufacturing the field emission electron source is illustrated as the following steps: Step 1, providing a CNT array; Step 2, drawing a number of CNT bundles from the CNT array to form a CNT yarn; Step 3, soaking the CNT yarn in an organic solvent, and shrinking the CNT yarn into a CNT string after the organic solvent volatilizing; Step 4, irradiating a predetermined point of the CNT string with a laser beam; Step 5, applying a voltage between two opposite ends of the CNT string, until the CNT string snaps; and Step 6, attaching the snapped CNT string to a conductive base, and achieving a field emission electron source.

In step 1, the CNT array is a super-aligned CNT array, which is grown using a chemical vapor deposition method. The method is described in U.S. Pat. No. 7,045,108, which is incorporated herein by reference. Firstly, a substrate is provided, and the substrate is a substrate of p type silicon or n type silicon. Secondly, a catalyst layer is deposited on the substrate. The catalyst layer is made of a material selected from a group consisting of iron (Fe), cobalt (Co), nickel (Ni), and their alloys. Thirdly, the substrate with the catalyst layer is annealed at a temperature in an approximate range from 300 to 400 degrees centigrade under a protecting gas for about 10 hours. Fourthly, the substrate with the catalyst layer is heated to approximately 500 to 700 degrees centigrade and a mixed gas including a carbon containing gas and a protecting gas is introduced for about 5 to 30 minutes to grow a super-

aligned CNTs array. The carbon containing gas can be a hydrocarbon gas, such as acetylene or ethane. The protecting gas can be an inert gas. The grown CNTs are aligned parallel in columns and held together by van der Waals force interactions. The CNTs array has a high density and each one of the CNTs has an essentially uniform diameter.

In step 2, a CNT yarn may be obtained by drawing a number of the CNT bundles from the super-aligned CNTs array. Firstly, the CNT bundles including at least one CNT are selected. Secondly, the CNT bundles are drawn out using forceps or adhesive tape, to form a CNT yarn along the drawn direction. The CNT bundles are connected together by van der Waals force interactions to form a continuous CNT yarn. Further, the CNT yarn can be treated by a conventional spinning process, and a CNT yarn in a twist shape is achieved.

In step 3, the CNT yarn is soaked in an organic solvent. The step is described in U.S. Pat. Pub. No. 2007/0166223, which is incorporated herein by reference. Since the untreated CNT yarn is composed of a number of the CNTs, the untreated CNT yarn has a high surface area to volume ratio and thus may easily become stuck to other objects. During the surface treatment, the CNT yarn is shrunk into a CNT string 12 after the organic solvent volatilizing, due to factors such as surface tension. The surface area to volume ratio and diameter of the treated CNT string 12 is reduced. Accordingly, the stickiness of the CNT yarn is lowered or eliminated, and strength and toughness of the CNT string 12 is improved. The organic solvent may be a volatilizable organic solvent, such as ethanol, methanol, acetone, dichloroethane, chloroform, and any combination thereof. A diameter of the CNT string 12 is in an approximate range from 1 to 100 microns ( $\mu\text{m}$ ), and a length thereof is in an approximate range from 0.1-10 centimeters (cm).

Referring to FIG. 6, the step 4 includes the following sub-steps:

In sub-step (1), the CNT string 12 is placed in a chamber 20. The chamber 20 includes a transparent window 202, an anode 208 and a cathode 210 therein. The anode 208 and the cathode 210 lead (i.e., run) from the inside to the outside of the chamber 20. Two opposite ends of CNT string 12 are attached to and electrically connected to the anode 208 and the cathode 210, respectively. In sub-step (2), a focused laser beam 30 radiates at a predetermined point 50 of the CNT string 12. The predetermined point 50 is located along a long-axial of the CNT string 12. The laser beam 30 projects through the window 202 and scans perpendicular to the long-axial of the CNT string 12. In the present embodiment, a power of the laser beam is 12 watts (W), and a scanning velocity thereof is 100 mm/S.

In step 5, a voltage is applied between the anode 208 and the cathode 210 to apply a voltage on the CNT string 12. The voltage is determinated according to a diameter and/or a length of the CNT string 12. In the present embodiment, the CNT yarn 12 is 2 cm in length and 25  $\mu\text{m}$  in diameter, and then a 40 voltage (V) DC bias is applied between the anode 208 and the cathode 210 to heat the CNT string 12 in air. After a while, the CNT string 12 is snapped at a predetermined point 50, and two snapped CNT strings 12 respectively having a broken end portion 124 are formed.

When the voltage is applied to the CNT string 12, a current flows through the CNT string 12. Consequently, the CNT string 12 is heated by Joule-heating, and a temperature of the CNT string 12 can reach an approximate range from 2000 to 2400 Kelvin (K). The resistance at the points distributing along the long axial of the CNT string 12 is different, and thus the temperature distributing along the long axial of the CNT string 12 is different. Due to the heat of the laser beam 30, the

CNT string 12 is oxidized at the predetermined point 50, some defects are formed thereat, and thus the resistance at predetermined point 50 increases. The greater the resistance and higher the temperature, the more easily snapping. In the present embodiment, after less than 1 hour (h), the CNT string 12 is snapped at the predetermined point 50.

The CNTs at the broken end portion 124 have smaller diameter and fewer number of graphite layer, typically, less than 5 nanometers (nm) in diameter and about 2-3 in wall. However, the CNTs in the CNT string 12 other than the broken end portion 124 are about 15 nm in diameter and more than 5 in wall. It can be concluded that the diameter and the number of the graphite layers of the CNTs decreases in a vacuum breakdown process. A wall by wall breakdown of CNTs is due to Joule-heating at a temperature higher than 2000K, with a current decrease process. The high-temperature process can efficiently remove the defects in CNTs, and consequently improve electric and thermal conductivity, and mechanical strength thereof. FIG. 7 shows a Raman spectrum of the broken end portion 124. After snapping, the intensity of D-band (defect mode) at  $1350\text{ cm}^{-1}$  is reduced, which indicates the structure effects at the broken end portion 124 are effectively removed, and thus the electric and thermal conductivity, and mechanical strength of the CNT string 12 are improved. Therefore, the field emission efficiency of the CNT string 12 is improved.

Moreover, during snapping, some carbon atoms vaporizes from the CNT string 12. After snapping, a micro-fissure (no labeled) is formed between two broken end portions 124, arc discharge may occur between the micro-fissure, and then the carbon atoms are transformed into the carbon ions due to ionization. These carbon ions bombard/etch the broken end portions 124, and then the broken end portion 124 form the tooth-shaped structure. Therefore, a shield effect caused by the adjacent CNTs can be reduced. The field emission efficiency of the CNT string 12 is further improved.

In step 6, the snapped CNT string 12 is attached to/electrically contacted with a conductive base 14. The end portion 122 of the CNT string 12 is attached to/electrically connected with a conductive base 14 by silver paste, the broken end portion 124 is a free end having the electron emitters, and then a field emission electron source 10 is formed.

FIG. 8 shows an I-V graph of the present field emission electron source. A threshold voltage thereof is about 250 V, an emission current thereof is over  $150\text{ }\mu\text{A}$ . The diameter of the broken end portion is about 5  $\mu\text{m}$ , and thus a current density can be calculated over  $700\text{ A/cm}^2$ . The inset of FIG. 8 shows a Fowler-Nordheim (FN) plot, wherein the straight line ( $\ln(I/V^2)$ ) via  $1/V$ ) indicate a typical field emission efficiency of the field emission electron source.

Finally, it is to be understood that the above-described embodiments are intended to illustrate rather than limit the invention. Variations may be made to the embodiments without departing from the spirit of the invention as claimed. The above-described embodiments illustrate the scope of the invention but do not restrict the scope of the invention.

What is claimed is:

1. A method for manufacturing a field emitter comprising: providing a CNT array; drawing a plurality of CNT bundles from the CNT array to form a CNT yarn; soaking the CNT yarn into an organic solvent, and shrinking the CNT yarn into a CNT string after the organic solvent volatilizes; irradiating a predetermined point of the CNT string with a laser beam, and forming an oxidized defect; applying a voltage between two opposite ends of the CNT string, until the CNT string snaps, wherein the snapped CNT string comprises a broken end portion, the broken

end portion comprises a plurality of CNT bundles, each of the plurality of CNT bundles has a taper shaped end comprising a plurality of CNTs, and some CNTs protrude from other adjacent CNTs; and

5. attaching the snapped CNT string to a conductive base, and achieving a field emission electron source.

2. The method as claimed in claim 1, wherein the predetermined point is located along the longitudinal axis of the CNT string.

10. 3. The method as claimed in claim 1, wherein the CNT string snaps at the predetermined point.

4. The method as claimed in claim 1, wherein the voltage is applied between the two opposite ends of the CNT string to heat the CNT string in air.

15. 5. The method as claimed in claim 1, wherein the CNT array is a super-aligned CNT array.

6. The method as claimed in claim 1, wherein the voltage is determined by a diameter and a length of the CNT string.

20. 7. The method as claimed in claim 6, wherein the diameter of the CNT string is in an approximately range from 1 micron to 100 microns.

8. The method as claimed in claim 6, wherein the length of the CNT string is in an approximately range from 0.1 centimeters to 10 centimeters.

25. 9. The method as claimed in claim 1, wherein the voltage is about 40 volts.

10. The method as claimed in claim 1, wherein upon applying the voltage, temperature of the CNT string reaches about 2000 to 2400 K.

30. 11. The method as claimed in claim 1, wherein a threshold voltage of the field emission electron source is about 250 volts, and an emission current of the field emission electron source is more than 150 microamperes.

12. The method as claimed in claim 1, wherein before soaking the CNT yarn into an organic solvent, the CNT yarn is treated by a spinning process.

35. 13. The method as claimed in claim 1, wherein a power of the laser beam is 12 watts, and a scanning velocity thereof is 100 mm/S.

14. A method for manufacturing a field emitter, comprising:

40. providing a CNT array; drawing a plurality of CNT bundles from the CNT array to form a CNT yarn; soaking the CNT yarn in an organic solvent, and shrinking the CNT yarn into a CNT string after the organic solvent volatilizes; irradiating a predetermined point of the CNT string with a laser beam; applying a voltage between two opposite ends of the CNT string to snap the CNT string at the predetermined point, and respectively forming two snapped CNT strings with a broken end portion and a micro-fissure between the two broken end portions; forming a tooth-shaped structure on the broken end portions, wherein the tooth-shaped structure comprises a plurality of CNT bundles, each of the plurality of CNT bundles has a taper shaped end comprising a plurality of CNTs, and some CNTs protrude further than other adjacent CNTs; and attaching the snapped CNT string to a conductive base, and achieving a field emission electron source.

45. 15. The method as claimed in claim 14, wherein the step of forming the tooth-shaped structure comprises a step of generating carbon ions transformed from carbon atoms during an arc discharge between the micro-fissure, and bombarding the broken end portions with the carbon ions.

UNITED STATES PATENT AND TRADEMARK OFFICE  
**CERTIFICATE OF CORRECTION**

PATENT NO. : 7,997,950 B2  
APPLICATION NO. : 12/006334  
DATED : August 16, 2011  
INVENTOR(S) : Yang Wei et al.

Page 1 of 1

It is certified that error appears in the above-identified patent and that said Letters Patent is hereby corrected as shown below:

**Title Page**

Please replace Section (73) regarding "Assignees" on the front page of the Patent with the following:

(73) Assignees: Tsinghua University, Beijing (CN), Hon Hai Precision Industry Co.,  
Ltd., Tu-Cheng, New Taipei (TW).

Signed and Sealed this  
Twenty-second Day of November, 2011



David J. Kappos  
*Director of the United States Patent and Trademark Office*